

# UNITED STATES PATENT OFFICE.

HANS GOLDSCHMIDT AND KARL MÜLLER, OF ESSEN, GERMANY, ASSIGNEES, BY MESNE ASSIGNMENTS, TO THE CHEMICAL FOUNDATION, INC., A CORPORATION OF DELAWARE.

## ZINC ALLOY.

1,358,147.

Specification of Letters Patent. Patented Nov. 9, 1920.

No Drawing.

Application filed April 19, 1917. Serial No. 163,262.

To all whom it may concern:

Be it known that we, HANS GOLDSCHMIDT and KARL MÜLLER, doctors of chemistry, citizens of the German Empire, residing at 5 Essen, Province of the Rhine, Germany, Salkenbergsweg 18, have invented a new and useful Improvement in Zinc Alloys; and we do hereby declare the following to be a full, clear, and exact description of the same.

10 The object of our invention is an alloy of zinc and aluminum containing manganese. By alloying zinc (for which purpose commercial spelter containing lead may be 15 used) with an amount of aluminum not considerably higher than is necessary for forming the eutectic mixture zinc-aluminum, that is to say 5.3 per cent. of aluminum, alloys are obtained which can be forged and rolled 20 within certain limits of temperature. However such binary alloys of zinc and aluminum show the heavy drawback that they do not yield sound castings.

We have found that the tendency of such 25 binary alloys of zinc and aluminum for forming blow-holes or pipes and for segregating is removed by adding a small amount of manganese. In this way alloys are obtained which yield dense and perfectly 30 homogeneous castings with a very small shrinkage. It may be remarked that by the addition of manganese the mechanical properties of these alloys, especially of the finished rolled material, are considerably

improved. Besides, such castings are better 35 worked than pure alloys of zinc and aluminum or than pressed zinc. The amount of aluminum has an upper limit in the formation of the eutectic mixture which, as above stated is about 5.3% and a lower limit 40 at about .5 per cent., whereas the addition of manganese may be varied from about .25 per cent. up to an amount not essentially exceeding 2 per cent.

The new alloys can be used as bearing- 45 metal and white-metal, furthermore for casting machine-fittings, for fuses and for rolled products.

• What we claim is:

1. An alloy of zinc containing from about .5% to about 6% aluminium and from about .25% to about 2% manganese.
2. An alloy of zinc containing from about .5% to about 6% aluminium and from about .25% to about 2% manganese, the content of 55 manganese being always less than the aluminium content.

3. A alloy of zinc containing about 5% aluminium and about 2% manganese.

In testimony whereof, we have signed our 60 names to this specification in the presence of two subscribing witnesses.

HANS GOLDSCHMIDT.  
KARL MÜLLER.

Witnesses:

FRANCES M. NUFER,  
FREDERICK J. DIETZMAN.